

## UNITED STATES PATENT OFFICE

2,340,726

## QUENCHING OF METALS

Clifford G. zur Horst, Hampton Township, Allegheny County, Blaine B. Wescott, Churchill Borough, and Leslie W. Vollmer, Pittsburgh, Pa., assignors to Gulf Research & Development Company, Pittsburgh, Pa., a corporation of Delaware

No Drawing. Original application January 12, 1942, Serial No. 426,537. Divided and this application July 13, 1943, Serial No. 494,532

6 Claims. (Cl. 148—13.1)

This invention relates to the quenching of metals; and it is particularly concerned with improved quenching oil compositions comprising a mineral quenching oil and an oil-soluble cumarone-indene resin in a controlled amount adequate to substantially increase the initial five second quenching speed without substantially modifying the stress-reducing characteristics of the oil; and it further comprises an improved process of quenching metals comprising pre-heating the metal to a temperature above its critical temperature and cooling the metal by immersion in a quenching oil bath comprising a light mineral quenching oil and 1.0 to 20.0 per cent of a cumarone-indene resin; all as more fully hereinafter set forth and as claimed.

While our invention is useful in the quenching of any metal which is advantageously quenched in an oil bath having a high initial quenching speed, it is particularly useful in the quenching of iron base alloys and it will be described hereinafter in detail in connection with the quenching of steel.

Many metal alloys, particularly iron base alloys, such as carbon steels and alloy steels, require heat treatment for the development of maximum properties of hardness and strength. These properties are dependent upon the establishment of certain physical structures in the metallic components of the alloy. In steel, hardenability is determined by the extent to which a martensitic structure is established in the alloy. The production of this structure in steel is usually accomplished by arresting at the desired point, the changes in the internal structure of the alloy which take place during the cooling of the steel from high temperatures. The fact that these physical changes require time for their completion makes it possible to arrest them at the desired point by suitable quick cooling.

Quenching of the steel in aqueous or oil quenching baths is generally used to arrest these physical changes. It is advantageously carried out in such manner that the physical changes in the steel are arrested at or near the point at which maximum hardness is obtained, and is then followed by a tempering treatment involving heating at relatively low temperatures to impart the desired ductility or toughness to the metal at some sacrifice in hardness.

Quenching in aqueous quenching media develops the properties of strength and hardness to the maximum obtainable for a given section of metal. However, quenching in aqueous quenching media is undesirable in many cases because these media tend to set up excessive amounts of internal stress in the steel resulting in distortion and warping and, in the extreme case, cracking of the quenched piece. As a result, aqueous quenching media have been supplanted by mineral oil quenching media where such mineral oil quenching media have sufficiently high quenching speeds to produce the desired properties in the quenched metal because such mineral oil quenching media are particularly adapted to minimize internal stresses and distortion in the quenched product. This results from the fact that the quenching speeds of mineral oil quenching media are substantially slower than those of aqueous quenching media, due to considerable extent to the formation of a more or less persistent vapor envelop about the quenched piece at the beginning of the quenching cycle, and the fact that in the later stages of the quenching cycle the quenching speeds of mineral oil quenching media are sufficiently slow so that the internal stresses developed in the metal in the early stages of the cycle tend to be relieved.

However, since the overall cooling efficiency of the mineral oil quenching media heretofore known is not as great as that of aqueous quenching media, it has been difficult or impossible to effect in mineral oil quenching baths quenching of pieces formed of steels having high critical cooling rates, sufficiently rapidly to develop the properties of strength and hardness to their maximum values or the quenching of pieces having high mass to surface ratios sufficiently rapidly to develop the properties of hardness and strength to the maximum depth.

It is desirable, therefore, to improve the quenching of metals in mineral oil quenching media so that the cooling efficiency in the early stages of the quenching cycle is increased to more nearly approach the cooling efficiency of aqueous quenching media without increasing the quenching speed in the later stages of the cycle sufficiently to deleteriously affect the normal stress-relieving properties of the mineral oil.

It is an object achieved by the present invention to provide a method of quenching metals, particularly iron base alloys, in mineral oil quenching media having initial quenching speeds greater than the mineral oil quenching media heretofore known.

It is a further object achieved by the present invention to provide mineral oil quenching compositions having cooling efficiencies more nearly approaching the cooling efficiency of water while retaining the stress-preventing characteristics of oil quenches.

The critical cooling rate of a metal is defined as the lowest cooling rate at which maximum hardness is developed. For steel the critical cooling rate is the lowest cooling rate which will produce a full martensitic structure in the steel. Thus it is generally most desirable to effect initial quenching at a speed sufficient to produce a cooling rate at least equal to the critical cooling rate for as great a depth in the metal as possible and to effect the quenching with a minimum of distortion.

The cooling efficiency of a quenching medium is customarily defined in terms of quenching speed and the initial five second quenching speed is a convenient measure of this property of quenching oil compositions, and is the property with which this invention is most concerned. The initial five second quenching speed of a quenching oil composition as referred to throughout this specification and in the appended claims is determined according to the following formula:

$$\frac{\text{Temperature rise in 5 sec. test}}{\text{Temperature rise in cold quench test}} \times 100 = \frac{\text{Per cent available heat removed in first five seconds}}{\text{seconds}}$$

in which the respective values are measured as follows:

Cylindrical test pieces one inch in diameter and 2.5 inches long of stainless steel containing about 18.0 percent of chromium and 8.0 per cent nickel are heated for one hour at 1500° F. in a furnace equipped with an automatic temperature control. Two quarts of the quenching oil composition to be tested are placed in a calorimeter which has a wire screen positioned in the center of the oil bath to insure constant depth of immersion of the samples. The quenching composition is heated to an initial temperature of 100° F.

One of the preheated test pieces is immersed in the quenching bath by means of light tongs for a period of five seconds without agitation. The test piece is then removed and the bath agitated and the maximum temperature reached is measured. A second preheated test piece is immersed in the bath at an initial temperature of 100° F. and the bath is agitated until the maximum rise in temperature has been produced. The maximum temperature rise measured in this cold quench represents the available heat of the test piece. By substituting the values thus determined for the five second quench and for the cold quench in the above formula, a measure of the heat removed in the first five seconds as compared with the total available heat is obtained and is referred to herein as the initial five second quenching speed.

We have discovered that oil-soluble cumarone-indene resins have the property, when incorporated in a light mineral oil such as has been used heretofore in the quenching of metals, of substantially increasing the initial five second

quenching speed of such an oil without lessening its stress-reducing characteristics, and that by incorporating such synthetic resins in mineral quenching oils even in amounts as small as 1.0 per cent substantial increases in the initial five second quenching speeds of the oils can be produced. Furthermore, we have found that the addition of the cumarone-indene resins to the mineral quenching oils does not deleteriously affect the stress-relieving properties which normally characterize such oils. By quenching pieces formed of metals having high critical cooling rates or pieces difficult to quench because of a high ratio of mass to surface, by immersion in quenching oil compositions containing these cumarone-indene resins, cooling of the metal can be effected at a rate more nearly approaching or equal to the critical cooling rate of the metal without creating excessive stresses in the metal. In this way the hardness of metal having high critical cooling rates can be developed to a degree heretofore unattainable with mineral oil quenching media, and hardening can be effected to a greater depth in pieces having high ratios of mass to surface. Both of these results can be achieved with a minimum of distortion.

The cumarone-indene resins which have been found useful for the purpose of our invention are customarily prepared commercially by the polymerization of the cumarone and indene components of coal-tar naphtha fractions. The starting material is usually a sharply fractionated naphtha boiling between 160° and 180° C., which has been treated for the removal of such impurities as naphthalene and phenols. Various polymerization catalysts may be used such as sulfuric acid, stannic chloride and anhydrous phosphoric acid. However, in substantially all commercial operations sulfuric acid is used in amounts corresponding to about 0.2 to 1.0 per cent by volume of 66° Bé. acid. The polymerization is highly exothermic and the batch should be kept below about 20° C. usually at 0° to 15° C. Dilution of the naphtha with petroleum distillate is sometimes resorted to in order to minimize overheating. The use of petroleum distillate in this manner also has the advantage that it has a solvent action on the desired polymerized products while undesirable products are caused to precipitate. When petroleum distillates are not present during the polymerization, they may be used to effect a separation of the polymerization products by dissolving out the resin polymer. After polymerization, tar and acid are settled out of the oil containing the cumarone-indene resin and the oil is neutralized with dilute caustic soda solution and is washed with water. The washed oil is then distilled off and the resin is recovered as a residue.

The properties of cumarone-indene resins can be varied by producing modified resins, for example such as are formed in the presence of alkyl ethers, phenols and the like. Properties can also be modified by formation of hydrogenated cumarone-indene resins. All of these cumarone-indene resin products have the property we have found of increasing the initial five second quenching speed of mineral oils and by the term cumarone-indene resins as used herein and in the appended claims we mean to include not only the resins which are obtained by the polymerization of cumarone and indene but also the modified and hydrogenated cumarone-indene resins.

Among the cumarone-indene resins with which we have obtained good results according to this

invention are resins exhibiting the following properties:

Table

|                            | C-I resin A      | C-I resin B         |
|----------------------------|------------------|---------------------|
| Melting range.....°C.      | 145-155          | 150                 |
| Ash.....per cent           | 0.1              | 0.1                 |
| Acid number (max.)         | 0.34             | 1.0                 |
| Saponification number..... | Not saponifiable | Not saponifiable    |
| Iodine number.....         | 30               | 45                  |
| Specific gravity.....      | 1.05             | 1.15                |
| Oil solubility.....        | Complete         | Complete at 100° F. |

The cumarone-indene resins, when incorporated in amounts corresponding to about 1.0 to 20.0 per cent by weight in mineral oils such as have been used heretofore in the quenching of metals, produce quenching compositions having quenching speeds of at least about 20.0 per cent.

The various cumarone-indene resins contemplated by the present invention do not increase the initial five second quenching speed of a mineral oil in the same degree. Some are more effective than others and also some are more oil-soluble than others and may be used in larger amounts. We have found also that in most cases the effect of each cumarone-indene resin increases directly with the amount used up to a maximum and then decreases. Consequently, the optimum range of concentration for different cumarone-indene resins will differ. In general, however, we have found that amounts between about 1.0 and 20.0 per cent by weight effect substantial increases in the initial five second quenching speed of an oil. By use of the proper resin in suitable amount substantially any initial 5 second quenching speed between about 20.0 per cent and 37.0 per cent can be obtained. It is possible, therefore, by suitably compounding quenching oil compositions according to our invention to provide a quenching medium which has an initial five second quenching speed particularly adapted to give best results with the particular metal and the particular type of piece being quenched. For most purposes it is advantageous to use a quenching composition having an initial five second quenching speed of at least about 30.0 per cent and for this reason we find it most advantageous to use the cumarone-indene resins in amounts corresponding to at least about 3.0 per cent by weight of the oil.

In compounding the quenching oil compositions of our invention we select for the quenching bath a mineral oil of the type customarily used for quenching steel and other metals and these oils are referred to herein as mineral quenching oils. The oils used for this purpose may be either naphthenic or paraffinic oils and are usually acid treated neutral oils having a viscosity of about 70 to 200 S. U. V. at 100° F., relatively high flash and fire points, and substantial heat stability and resistance to sludging. For optimum results we have found that paraffinic oils which usually have an initial five second quenching speed between about 17.0 and about 19.0 per cent are most advantageous.

We have found also that mixtures of the quenching accelerating agents of our invention may be used. However, in such case, the effect of the respective agents is not entirely additive and the optimum amounts of the respective agents, when used alone, may produce less satisfactory results in mixtures than do somewhat smaller amounts of each agent.

The actual quenching operation using the

quenching compositions of our invention is usually carried out by immersion of the preheated metal in the quenching oil composition until sufficient heat has been removed to reduce its temperature the desired amount. The quenching oil may be used repeatedly with only slight deterioration.

In the following examples there are illustrated specifically several of the more advantageous forms of our invention and the results obtainable thereby.

*Example 1.*—The following test results illustrate the use of cumarone-indene resins according to our invention.

A series of quenching oil compositions was prepared by mixing a hydrogenated cumarone-indene resin having the properties shown above in the table for resin A in amounts between 1.0 and 15.0 per cent by weight, respectively, with a neutral paraffinic mineral oil having a viscosity of 100 S. U. S. at 100° F. The initial five second quenching speeds of the respective compositions were then measured as above described and the following results were obtained:

|                                           | Initial five second quenching speed |
|-------------------------------------------|-------------------------------------|
| Quenching oil No. 2.....                  | 18.98                               |
| Quenching oil+1.0% cumarone-resin A.....  | 20.16                               |
| Quenching oil+2.0% cumarone-resin A.....  | 24.66                               |
| Quenching oil+3.0% cumarone-resin A.....  | 31.26                               |
| Quenching oil+4.0% cumarone-resin A.....  | 33.20                               |
| Quenching oil+5.0% cumarone-resin A.....  | 34.36                               |
| Quenching oil+7.5% cumarone-resin A.....  | 35.93                               |
| Quenching oil+10.0% cumarone-resin A..... | 36.81                               |
| Quenching oil+12.5% cumarone-resin A..... | 36.83                               |
| Quenching oil+15.0% cumarone-resin A..... | 36.32                               |

As will be seen from these results, this hydrogenated cumarone-indene resin is a very effective quenching accelerating agent. Also, it will be observed that the increase in initial five second quenching speed with increased amounts of resin passes through a maximum.

Another series of quenching oil compositions was prepared by mixing a cumarone-indene resin having the properties shown above in the table for resin B, in amounts corresponding to 1.0 to 5.0 per cent by weight, respectively, with the same neutral paraffinic oil of 100 S. U. S. at 100° F. The initial five second quenching speeds of the oil-resin compositions were determined as outlined above. The results obtained are as follows:

|                                          | Initial five second quenching speed |
|------------------------------------------|-------------------------------------|
| Quenching oil No. 2.....                 | 18.98                               |
| Quenching oil+1.0% cumarone-resin B..... | 21.22                               |
| Quenching oil+2.0% cumarone-resin B..... | 25.39                               |
| Quenching oil+3.0% cumarone-resin B..... | 32.42                               |
| Quenching oil+4.0% cumarone-resin B..... | 35.01                               |
| Quenching oil+5.0% cumarone-resin B..... | 35.81                               |

These results also demonstrate the effectiveness of the cumarone-indene resins as quenching accelerating agents.

Hardness and distortion tests were made on pieces of metal quenched in the oil composition containing 5.0 per cent of this cumarone-indene B. These measurements were made on specially designed pieces adapted to show, measurably, very small changes in shape due to distortion and having a continuously changing section which permitted measurement of the variation in surface hardenability with varying section of the piece and thereby gives an indication of the vari-

ation in depth of hardening of the piece. The changes in shape were measured in inches and the maximum Brinell hardness occurring at different points on the surface of the piece were determined. Comparative tests were made on pieces quenched in water and in the mineral oil alone.

Results of the distortion measurements are shown in the following table:

| Quenching medium                  | Dimension A | Change in dimension, B | Dimension C |
|-----------------------------------|-------------|------------------------|-------------|
| Tap water.....                    | +0.0134     | +0.0102                | +0.0116     |
| Oil No. 2.....                    | +0.0032     | +0.0024                | +0.0028     |
| Oil No. 2 and 5% C-I resin B..... | +0.0020     | +0.0041                | +0.0041     |

Results of the hardness measurements are shown in the following table:

| Quenching medium                  | Brinell hardness |         |           |
|-----------------------------------|------------------|---------|-----------|
|                                   | Minimum          | Maximum | Variation |
| Tap water.....                    | 649              | 723     | 74        |
| Oil No. 2.....                    | 361              | 696     | 335       |
| Oil No. 2 and 5% C-I resin B..... | 573              | 720     | 147       |

From these results it will be observed that while tap water gives the greatest surface hardness and a variation of only 74 points from the hardest to the softest area, it also gives maximum distortion. The mineral oil alone minimizes distortion but gives a lowered surface hardening and a variation of 335 points from the hardest to the softest point. On the other hand, the specimen quenched according to our invention in a quenching oil composition having an initial five second quenching speed of about 35.8 per cent showed distortion approximately equal to that obtained with plain mineral oil, a surface hardness almost equal to that obtained with water and a hardness variation little greater than that obtained with water and substantially less than that obtained with oil alone, indicating a depth of hardening intermediate between those obtained with water and with oil alone, respectively.

This application is a division of our copending parent application Serial No. 426,537, filed January 12, 1942.

While we have particularly described our in-

vention with reference to certain specific embodiments thereof, it is to be understood that it is not limited to such specific embodiments except as hereinafter defined in the appended claims.

What we claim is:

1. An improved quenching oil composition comprising a mineral quenching oil and at least about 1.0 per cent by weight of an oil-soluble cumarone-indene resin.

2. An improved quenching oil composition comprising a mineral quenching oil and an oil-soluble cumarone-indene resin in controlled amount adequate to impart to said quenching oil an initial five second quenching speed of at least about 20.0 per cent without substantially modifying the stress-reducing characteristics of the oil.

3. A method of quenching metals comprising heating the metal to a temperature above its critical temperature and thereafter cooling the metal by immersion in a quenching oil bath comprising a mineral quenching oil and an amount of an oil-soluble cumarone-indene resin, above about 1.0 per cent adequate to impart to the quenching oil bath an initial five second quenching speed of at least about 20.0 per cent.

4. An improved quenching oil composition comprising a solution of at least 3.0 per cent by weight of an oil-soluble cumarone-indene resin in a mineral quenching oil.

5. An improved quenching oil composition comprising a mineral quenching oil and a cumarone-indene resin in a controlled amount adequate to impart to said quenching oil an initial five second quenching speed of about 30.0 to 37.0 per cent without substantially modifying the stress-reducing characteristic of the oil.

6. A method of quenching metals comprising heating the metal to a temperature above its critical temperature and thereafter cooling the metal by immersion in a quenching oil bath comprising a mineral quenching oil and an amount of an oil-soluble cumarone-indene resin above about 3.0 per cent adequate to impart to the quenching oil bath an initial 5 second quenching speed between about 30.0 to 37.0 per cent.

CLIFFORD G. ZUR HORST.  
BLAINE B. WESTCOTT.  
LESLIE W. VOLLMER.